

## UNITED STATES PATENT OFFICE

2,221,232

PRODUCTION OF CREPELIKE TEXTILE  
WEBS

René Clavel, Augst, near Basel, and Theophil Stanisz, Basel, Switzerland, assignors to Farberei-und Appretur-Gesellschaft Vorm. A. Clavel und Fritz Lindenmeyer, Basel, Switzerland

No Drawing. Application August 17, 1937, Serial No. 159,602. In Germany April 22, 1937

5 Claims. (Cl. 8—114)

Acetate artificial silk (cellulose acetate silk) textile webs having crepe effects have hitherto only been produced in practice by using highly twisted threads. This relatively expensive process only enables crepe effects of a simple kind to be produced and is not suitable for the production of webs having numerous variations or for the production of cloque effects and the like.

The object of this invention is to produce acetate artificial silk textile webs having a lustrous or dull finish and provided with crepe effects with the employment of untwisted or only slightly twisted acetate threads.

The invention depends on the fact that it is possible on the one hand by treating acetate silk threads with suitable chemicals to cause them to shrink to a desired, even very considerable, degree, and the fact that on the other hand it is possible so to protect the acetate silk threads by treatment with suitable protective substances (reserves), that they do not undergo shrinkage by the action of chemicals in themselves adapted to shrink acetate silk threads.

According to this invention therefore by working up protected and untreated acetate silk threads together it is possible to produce products of the desired kind by treating the same with shrinking agents, which cause the untreated acetate silk threads to shrink and thereby to produce the most varied crepe effects and the like, owing to the non-shrinkage of the protected threads.

As protective agents (reserves) for the acetate silk threads use is preferably made of phenols, which contain free active OH groups, i. e. possess a phenolic character, for example tannin and tannin-like substances, such as catechol. These may be employed in the form of aqueous solutions; if necessary, small quantities of swelling agents, such as concentrated formic acid, may be added to the solutions. Synthetic products, for example condensation products of phenols with aldehydes, for example formaldehyde, which can be converted by sulphonation, preferably weak sulphonation, into a water-soluble condition, may also be employed as protective agents. In general there may be employed as protective agents substances, which contain active groups, which, as for example OH groups, are capable of being fixed by the cellulose acetate. In this way protective effects based on chemical reactions may be obtained. Such compounds, for example condensation products of phenol and resorcinol with formaldehyde, may also be employed in a sulphonated

condition in the form of suitable emulsions or suspensions, resembling the dyestuff emulsions employed for the dyeing of acetate silk.

As shrinking agents use is preferably made of acid liquids of suitable concentrations, which do not attack the cellulose acetate under the working conditions, for example about 23–26% hydrochloric acid, about 60–68% phosphoric acid or about 38–48% acetic acid. In addition to inorganic and organic acids, alkali and alkaline earth thiocyanates may also be employed inter alia as shrinking agents. The shrinking agents must be employed at moderate temperatures, preferably temperatures not exceeding about 20° C., for example at a room temperature of about 18 to 20° C. The length of treatment must be such that the cellulose acetate is not attacked to any destructive extent. As a rule a working period of a few minutes suffices.

The following example serves to illustrate how the process of this invention may be carried into effect:

Acetate silk in hank form is saturated with an aqueous solution which contains about 200 gms. of tannin, 10 gms. of concentrated formic acid and 790 gms. of water per litre, in order to protect it from shrinking. The acetate silk is treated in the cold, centrifuged, dried and if necessary treated for a short time longer with steam under pressure, for example is steamed for about 15 minutes in a closed vessel at about 108° C., in order to effect thorough fixing.

After the treatment with protective agents, the acetate silk is advantageously treated with a suitable dressing solution, for example an approximately 3% wax and paraffin solution in organic solvents, such as benzine, benzene and the like. The threads are thereby rendered more adaptable for further treatment, for example weaving. It is also advisable slightly to dye the threads, which may be effected in a very simple manner by adding suitable dyes to the dressing solution. This offers the advantage that the slightly dyed threads can be readily distinguished from the untreated threads during the subsequent operations.

In the process of weaving, the protected threads and the untreated acetate silk threads may be woven in the weft or warp or both. The most varied effects may be obtained by varying the arrangement of the protected threads and the untreated threads relatively to one another and the relative proportions of the protected threads to the untreated threads. In general it has proved to be advantageous to employ in the

weft or the warp or in both about 5-10 protected threads to about 3-8 untreated threads.

The webs produced from protected and untreated threads by weaving or the like are then 5 treated with shrinking agents, preferably acid shrinking agents, the working conditions, for example with regard to concentration of the solution, time of treatment and temperature being so selected, that on the one hand shrinkage of 10 the untreated threads to the desired degree takes place, whilst on the other hand the cellulose acetate is not attacked or otherwise influenced to a destructive extent. Shrinking effects from about 10% to about 50% may be obtained according to the invention in the weft and the 15 warp, depending on the conditions selected. Depending on the degree of shrinkage of the untreated threads, the protected, non-shrinking threads or thread parts are more or less raised 20 and thereby more or less pronounced crepe effects are produced.

The treatment of the fabric with the shrinking liquid, for example about 25% hydrochloric acid, is for example carried out as follows:

25 The pieces, bands or the like are left for up to 5 minutes in the acid at a temperature which must not exceed 20° C., for example at a room temperature of about 18° C., then freed in a loose condition from adhering hydrochloric acid, for 30 example by washing in a container with flowing water and are then with advantage further subjected to an after-treatment in a weak alkaline liquid for example in a bath which contains a solution of 3 gms. of sodium carbonate per litre, in 35 order to effect neutralisation. If desired the reserves may at the same time be removed from the threads by this alkaline after-treatment. In order to achieve this result the operation is with advantage carried out at elevated temperatures, 40 for example temperatures of about 40-50° C. The removal of the reserves may also be effected with other agents, for example soap lyes.

The drying of the pieces is with advantage effected by allowing them to shrink unhindered 45 in a loose condition on suitable bases, for example tables. The pieces may be allowed to dry slowly at room temperature or slightly elevated temperature or they may be subjected to more rapid drying by the action of higher temperatures, 50 for example temperatures up to about 90° C.

The process may with advantage be carried out with the employment or co-employment of the so-called continuous apparatus. The treatment of the pieces with aqueous hydrochloric acid may for example be carried out in accordance 55 with the continuous process, care being taken in this case also to ensure that they do not stay for more than about 5 minutes in the acid solution, since otherwise the hydrochloric acid might exert a disturbing effect. The drying 60 may likewise take place in accordance with the continuous process, for example by bringing the pieces in a loose condition on to an endless belt onto which hot air is blown. Alternatively 65 the endless belt may be passed through a hot chamber, through which for example hot dry air is circulated.

It is essential, during the hydrochloric acid treatment and the following wet and dry treatments, to avoid stretching, particularly considerable stretching, of the web. This is particularly the case when employing the continuous process. Drying on rods must be avoided, because the fabric is easily stretched thereby and 75 the crepe effects, designs, etc. may be distorted.

Crepe effects may for example be obtained by the process of this invention by using only protected and untreated acetate silk threads for the warp and only ordinary (untreated) or only protected threads for the weft. Similarly crepe effects may for example be obtained by using only ordinary (untreated) acetate silk threads or only protected threads for the warp and desired combinations of protected and untreated threads for the weft. Particularly pronounced crepe effects 10 are obtained by using ordinary threads and protected threads for the warp and weft in suitable arrangements and proportions.

By employing a relatively large number of untreated threads in addition to a relatively small 15 number of treated threads, so-called faconnet effects (striped effects) may for example be obtained in a very simple manner. In order to obtain special effects, the threads to be protected may for example be treated with weaker solutions, than are necessary for producing complete protection, or different threads may be treated with protective solutions of different strengths or one and the same thread may be treated in different parts with protective solutions of different strengths. A further alternative when protecting hanks of threads is for example to treat these hanks only in parts with the protective solution, so that in the treatment of the fabric with shrinking liquids these threads remain unchanged in the protected parts and shrink in the unprotected parts.

So-called cracknel effects may for example also be obtained by twisting together protected acetate silk threads and untreated threads and then weaving or knitting the twisted threads. On treating the resulting products with shrinking liquids, the unprotected threads are shortened and thereby the cracknel effect is obtained.

Further researches have shown that in place of 40 the acetate silk threads protected according to the invention textile threads of other kinds may be employed or co-employed with protected acetate silk threads. It has been found that threads of for example natural silk (schappe), wool, cotton, linen, cellulose artificial silk and other natural and artificial textile threads, when subjected to the process of this invention, behave in the same manner as protected acetate silk threads, in that during the treatment of the mixed fabric with liquids which shrink ordinary (untreated) acetate silk threads, they undergo no shrinkage or no detrimental shrinkage. Thus fabrics and the like products may be manufactured with the production of crepe effects of the 45 most varied kinds, by effecting the formation of the crepe patterns by shrinking ordinary (untreated) acetate silk threads whilst the remaining threads, which do not or only in part participate in the shrinking processes, may consist of other textiles of the most varied kinds, if desired a plurality of such textiles. Accordingly mixed webs of cellulose acetate threads and other kinds of threads, for example natural silk, wool or cotton threads, if desired a plurality of such threads, may accordingly be produced in a very 50 simple manner and in this way special effects be obtained. In all cases undyed, dyed or partially dyed products having a lustrous or dull finish, may be produced, such as it has hitherto 55 not been possible to produce with the aid of twisted acetate silk threads.

According to one embodiment of this invention the procedure is followed of printing woven textiles produced from acetate artificial silk with 75

reserves, which effect suitable protection against shrinkage, and then subjecting the printed textiles to the shrinking process with the use of suitable shrinking agents, for example about 25% hydrochloric acid. In this way it is possible to print designs of the desired kind on the materials under treatment by the usual methods, for example with the aid of printing machines, stencils or by hand, and thereby to protect the printed parts against shrinkage.

Protective agents of the aforesaid kinds, such as tannin or tannin-like substances, may also be employed in this case as reserves. When using the solutions for printing, they are adjusted to the desired degree of viscosity, for example with the aid of gum arabic or gum Senegal.

A reserve adapted for machine printing may for example have the following composition:

200 gms. of commercial tannin, 100 gms. of 20 50% acetic acid, 150 gms. of water and 550 gms. of gum.

For carrying out the printing process use may also be made of mechanically acting protective substances, for example natural or synthetic resins, waxes, paraffins and the like, for example an approximately 75% solution of colophony in organic solvents, such as xylene.

In this case also the webs after application of the reserves and drying may be steamed in order to improve the fixing.

The treatment of the webs with shrinking agents may be effected in the hereinbefore described manner. By the action of the shrinking agent the non-protected parts of the materials are swollen and shrunk and the fibres shortened. It is consequently possible to produce in a very simple manner special effects, such as patterns in relief or crepe designs.

In this embodiment of the invention also fabrics may be employed, which, in addition to cellulose acetate threads, also contain threads of other kinds. Similarly, webs may be employed, which, in addition to ordinary (untreated) acetate threads, also contain acetate threads protected according to the invention in the warp or weft or both. Finally the webs may also contain ordinary acetate threads, protected acetate threads and threads of other kinds.

The acetate webs or acetate-containing webs, before or after printing with the reserves, may be dyed or printed with colours, or alternatively colours may be applied simultaneously with the printing of the reserves.

When employing coloured reserves, adjuvants, for example a little acetin, are with advantage added to the colour. Coloured varnishes are formed thereby, which during the treatment of the webs with shrinking agents, particularly acids, are extremely resistant thereto, are not removed during the treatment with shrinking agents and subsequent treatments and do not bleed during the shrinking operation on to the unprinted parts. The webs produced by printing may be treated in the usual manner, for example steamed, washed and finished.

The invention, as has been shown, enables the most varied kinds of effects to be produced, including those, which it was hitherto not possible to obtain with the simplest and cheapest means. The products produced according to this

invention may be treated by the usual methods, for example bleached, loaded, dyed and finished.

What we claim is:

1. Process for producing textile goods having a crepe effect including the steps of treating a fabric with hydrochloric acid of a strength of about 23-26% at temperatures of not above 20° C., said fabric consisting of threads or thread portions which become shortened by the action 10 of hydrochloric acid of about 26% and of threads or thread portions which have been rendered resistant to the action of hydrochloric acid by treatment with tannin, removing the hydrochloric acid, drying the fabric, the whole treatment 15 being for the purpose of shortening by the above recited treatment with hydrochloric acid the threads or thread portions which have not been rendered resistant.

2. Process for producing textile goods having 20 a crepe effect including the steps of treating a fabric with hydrochloric acid of a strength of about 23-26% at temperatures of not above 20° C., said fabric consisting of threads or thread portions which become shortened by the action 25 of hydrochloric acid of about 26% and of threads or thread portions which have been rendered resistant to the action of hydrochloric acid by treatment with tannin, the entire treatment being for the purpose of shortening by the above 30 recited treatment with hydrochloric acid the threads or thread portions that have not been rendered resistant.

3. A process for the production of textile products, such as textile webs, having crepelike effects, which comprises working up acetate silk threads, which have been protected by pre-treatment against shrinkage, with ordinary untreated acetate silk threads into the product, and treating the product with agents which cause the untreated acetate silk threads to shrink, the acetate silk threads to be protected against shrinkage being subjected to a treatment with natural tannin.

4. A process for the production of textile products, such as textile webs, having crepelike effects, which comprises working up acetate silk threads, which have been protected by pre-treatment against shrinkage, with ordinary untreated acetate silk threads into the product, and treating the product with agents which cause the untreated acetate silk threads to shrink, the acetate silk threads to be protected against shrinkage being treated with synthetic products containing active hydroxyl groups and natural tannin.

5. A process for the production of textile products, such as textile webs, having crepelike effects, which comprises working up acetate silk threads, which have been protected by pre-treatment against shrinkage, with ordinary untreated acetate silk threads into the product, and treating the product with agents which cause the untreated acetate silk threads to shrink, the agent which is employed for protecting the web 60 in places against shrinkage is a resin containing natural tannin.